

Patented Feb. 7, 1933

1,896,215

# UNITED STATES PATENT OFFICE

THEODORE F. BRADLEY, OF WESTFIELD, NEW JERSEY,

## GREASE RESISTANT PAPER

No Drawing.

Application filed August 31, 1927. Serial No. 216,781.

This invention relates to grease resistant carton board and process of making same, and relates particularly to grease resistant paper products intended for use with greasy foodstuffs and other similar articles.

In the preferred form of my invention I provide a coating solution or composition for carton board which is almost non-volatile at ordinary room temperature, that is, at approximately 70° F. and yet which dries quickly at slightly elevated temperatures, for example, at about 140° F. This is of particular importance where liquids of alleged toxic nature, such as, for example, benzol are employed, and also when improved flowing and working qualities are desirable. One of the features of the present invention comprises a method for reducing, and, in fact, practically or substantially eliminating all evaporation of benzol at ordinary room temperatures (65°-70° F.) from nitrocellulose solutions, although not preventing the evaporation when the temperature is elevated, such as when the coated materials are exposed to a mild heat as by being quickly passed through ovens, equipped with ventilating devices or solvent recovery systems. It is sufficient to minimize evaporation at room temperatures so that the coated paper and solutions which the workmen handle, will not produce poisoning, or result in a waste of solvents.

Attempts have been made to secure easy flowing and slow drying nitrocellulose solutions by utilizing extremely high boiling solvents of low volatility, such solvents as glycol diacetate, glycol and glycerol ethers and esters, benzyl acetate, and various other cellulose ester solvents of the same range of volatility having been considered. These vehicles are rather costly, and, furthermore, have the disadvantage of being somewhat too slow drying, even when the materials are oven dried. Under the present invention I effect much less expensive and generally more satisfactory results.

This invention, in the embodiment which I consider most practicable at the present time, involves the use of coating compositions preferably containing nitrocellulose and a compatible resin or balsam and having a solvent vehicle for nitrocellulose easily volatile at ordinary room temperatures, preferably with a diluent of like or the same general range of volatility, together with such a percentage of a wax as will prevent appreciable evaporation of said solvents and yet yield a surface finish substantially free from rings, pock marks, waxy finish, or other such irregularities commonly caused by excess wax. It has been found that waxes such as Japan and carnauba waxes are of but little value in accomplishing the object of this invention, except as they may exert a polishing effect; the most satisfactory results having been secured from mineral waxes, either paraffin or ceresin wax or ozocerite. Furthermore, definite proportions have been determined, the use of substantially greater amounts than those stipulated tending to reduce the gloss of the coatings and to produce rings, pock marks, waxy surfaces, and various other surface irregularities, while the use of substantially lesser amounts do not satisfactorily check evaporation at room temperatures.

Thus a nitrocellulose and resin coating composition may be made as follows:

### Example 1

|                              | Parts by weight |
|------------------------------|-----------------|
| Rosin ester                  | 40              |
| Dibutyl phthalate            | 90              |
| Low viscosity nitrocellulose | 75              |
| Butyl acetate                | 150             |
| Toluol                       | 150             |
| Ethyl alcohol                | 30              |
| Ceresin wax                  | 2               |

This composition contains solvents of medium volatility, does not dry readily at or

dinary room temperatures, and yet has been found to dry very rapidly when surfaces coated with it are placed in an oven at about 120° to 140° F. The composition has been 5 found to dry to a flexible and glossy smooth surface. In manufacturing such a composition the wax and resin may be dissolved in a portion of the solvent mixture and blended with the nitrocellulose to form a clear solution.

Various other types of resins may be employed such as are commonly used in nitrocellulose compositions, including all of the usual natural resins, as well as such synthetic 15 resins as benzoic phthalic glyceride resin, rosin phthalic glyceride resin, Congo rosin phthalic glyceride resin, castor oil phthalic glyceride resin, and also a special type of resins produced from cottonseed oil fatty 20 acids, phthalic anhydride and glycerol. Although, as aforesaid, various resins may all be employed in the grease resistant compositions of this invention, it is advantageous and usually preferable to employ a resin 25 which is insoluble in fatty oils and greases. In fact, in case such a resin is employed, it is often possible to utilize only this resin as a greaseproofing agent, it being then not always necessary to employ nitrocellulose or 30 other cellulose ester. A suitable resin for this work is that which may be made by slowly heating 50 parts by weight of glycerol, 80 parts by weight phthalic anhydride and 45 parts by weight of the fatty acids of cottonseed oil to a temperature of 475° F. Since 35 this resin is somewhat soft, it is preferably used in combination with nitrocellulose when non-tacky surfaces are desired. Compositions may contain the various types of plasticizing agents such as castor and rapeseed 40 oils. In some cases all resin may be omitted. Various other types of plasticizing agents may be employed, or mixtures thereof, among which are castor and rapeseed oils, dibutyl 45 and diethyl phthalate, tricresyl phosphate, camphor and other nitrocellulose softening or plasticizing agents. Pigments may be employed if colored surfaces are desired.

Various solvents may be employed in the 50 production of the grease-resistant carton board. All of the usual nitrocellulose solvents of a low or medium volatility may be employed, it merely being necessary that said solvents or mixtures thereof have sufficient 55 solvent action on the wax to maintain the same substantially in solution; sufficient to function in the manner aforesaid. Thus, either ethyl, propyl, butyl, amyl and hexyl acetates or propionates may be used, in some 60 cases alone, or more preferably in admixture with various alcohols or hydrocarbon diluents of like degree of volatility. Other nitrocellulose solvents such as acetone, ethyl methyl ketone and similar volatile solvents 65 may likewise be employed to produce satis-

factory solvent vehicles. The proportion of wax may be altered slightly, according to the solvent mixture employed, although it is in all cases necessary that sufficient wax be used to render satisfactorily slow drying at room temperatures, while avoiding the use of such excessive amounts as will disrupt the surface finish. This will vary slightly according to the solvent mixtures employed and also according to such variations in room temperature as may obtain. In general, it is not advisable to employ substantially over 2 per cent (on the weight of the solvents employed) of paraffin or ceresin wax. A large proportion of wax, as stated, tends to produce defective surface finishes. Nor is it advisable to use much less than 1/2 of 1 per cent of said waxes. Less wax can be used in cold weather to good advantage in some cases. The use of alcohols have been found of some value 80 in reducing the viscosity of the nitrocellulose solutions for the purposes of the present invention. Replacement of 100 parts of toluol with a like amount of butyl alcohol, for example, gives lowered viscosity. The wax content then may be 1 or 1 1/2 instead of 2 parts.

It has been proposed to employ wax in paint and varnish removing compositions to retard evaporation, but in such compositions the proportion of wax is not confined to very narrow limits. Whereas, in my compositions a limitation is placed on the wax content such as to avoid surface defacement. In my compositions the wax preferably is maintained almost entirely in solution or dispersion through the aid of the nitrocellulose functioning as a protective colloid. Furthermore, the present application relates to compositions which are intended for coating purposes, whereas the aforesaid paint and varnish removers are intended for the removal of coatings. In other words, my composition is intended for a totally different purpose than paint and varnish remover and is, moreover, prepared with respect to consideration of a character totally different from those obtaining in meeting the requirements of paint and varnish removers.

In the preferred form of my invention I employ volatile solvents which do not leave any disagreeable residual odor on paper surfaces treated therewith. While a single solvent such as acetone may be employed, it is preferable to use a composite one comprising a mixture of nitrocellulose solvent and wax solvent and containing a proportion of wax very slight with respect to the total amount of the composition, but sufficient to substantially prevent evaporation at 70° F., but not materially preventing evaporation at a temperature somewhat above 100° F.

To secure a maximum degree of wax-dispersing effect with a minimum of wax-expulsion with the object of eliminating surface

defacement by the wax, I preferably employ low viscosity nitrocellulose such as a grade above one second and below four second material. Low viscosity nitrocellulose has a 5 desirable cooperating action with the mineral wax or other wax employed. With such low viscosity nitrocellulose I may use a more effective concentration of wax and still keep the 10 proportion of wax below a surface-defacing concentration. This may be due to some species of protective colloid action or to other causes. Employment of low viscosity nitrocellulose in conjunction with a modicum 15 of wax in compositions intended for coating, constitutes a feature of the preferred form of my invention. An ultra-low-viscosity nitrocellulose such as one-half second or one-tenth second may be used in some cases.

I have set forth paraffin or ceresin wax in 20 the preferred compositions, and in general, have preference for a mineral wax; ceresin, because of its amorphous character being of particular value from the standpoint of effective dispersion and adequate proportion 25 at a concentration approaching the surface-defacing point. Beeswax and other waxes or mixtures of waxes, e. g., a mixture of beeswax and ceresin wax having properties like, or approaching the mineral waxes as set forth 30 herein are included within the purview of my invention, which embraces substances, a modicum of which greatly reduces evaporation 35 of the unitary or composite volatile solvent vehicle at room temperatures while permitting free escape thereof at slightly elevated 40 temperatures.

The proportions in the illustrative example may be varied and the components altered in 45 grade or quality as desired within wide limits (except as regards proportion of wax, as has been described). Some of the components are not essential at all times, and plasticizer, for example, may be omitted in some cases. The 50 resinous body likewise may be omitted if a pronounced gloss or strong adhesion is not needed. The foregoing has largely been derived from my co-pending patent application Serial No. 183,011 and constitutes a continuation 55 in part of the same.

Paper of various kinds such as manila, kraft, sulphite, tissue, glassine, carton board, and other types of paper are all subject to treatment by the process and with the compositions herein disclosed, in order to render 60 them substantially grease resistant and thus enable greasy food products to be contained therein without exudation of grease. The composition suitable for such use comprises either a grease-insoluble resin alone or more 65 preferably in admixture with nitrocellulose, acetyl cellulose, nitro-acetyl cellulose, cellulose ethers and/or organic-solvent-soluble cellulose compounds. When such cellulose compound is employed it is possible to incorporate other resins which are soluble in

grease in small proportions, although if a grease-insoluble resin such as the cottonseed phthalic glyceride synthetic resin is employed in admixture with nitrocellulose, it is possible to utilize very much larger percentages of the said grease-insoluble resin than of a grease-soluble resin. Thus, the composition utilized in the present invention embraces bodies which are substantially insoluble in grease or fatty oils, whether comprising a cellulose ester or a grease-insoluble resin. Utilizing either or both of these types of materials one may add thereto small proportions of grease-soluble materials as softening or extending agents without serious trouble.

#### Example 2

A composition containing a grease-resistant resin is the following:

|                                     | Parts by weight |
|-------------------------------------|-----------------|
| Low viscosity nitrocellulose        | 40              |
| Cottonseed phthalic glyceride resin | 40              |
| Dibutyl phthalate                   | 20              |
| Ethyl acetate                       | 135             |
| Benzol                              | 135             |
| Paraffin wax                        | 5               |

The paraffin wax is dissolved in a portion of the solvent vehicle and the nitrocellulose and synthetic resin are dissolved in other portions of the solvent vehicle, then admixed to form the finished coating composition. This may be thinned with the same solvent mixture to any desired extent, the exact amount of total solids being regulated to deposit the particular thickness of grease resistant coating desired. The composition may be applied by any suitable means to the paper which is to be treated. For the best result it is preferable to employ a paper having a surface easily impregnated and in some cases to secure the best impregnation it is desirable to conduct the coating operation under pressure. Ordinarily, however, the paper may be run over rolls or through a bath of the material, being coated on either one side or both as desired. The wax in the solution substantially checks the evaporation at room temperature, thus largely eliminating the poisoning hazard of benzol vapors, the coating material then being conducted into a closed drying system maintained at a somewhat elevated temperature, that is, at about 140° F. whereupon the coated material dries rapidly and the solvents may be forced out of the building or passed through a solvent recovery system, without danger to the workmen. Other suitable solvent vehicles comprise acetone in admixture with benzol, mixtures of ethyl acetate, benzol and denatured alcohol, etc. It is desirable to employ only such solvents as may be readily eliminated from the coated article and which do not

leave any residual odor to contaminate the paper so treated.

It has been found that coatings of this type are extremely resistant to penetration by oils and greases and also have a waterproofing action as well and that it is necessary to have a very good impregnation of the surface for proper protection. Very thin coatings of such degree of thickness that they can hardly be measured with a micrometer are often satisfactory, provided proper impregnation has been obtained. Surface coatings of great thickness are not usually so desirable, often being porous and of such different degree of flexibility from the paper that they often crack upon bending and separate from the paper surface. Thin layers show better adhesion to the paper surface and a greater degree of flexibility for a given composition than heavy papers. It is thus considered that a coating is not of optimum character unless a very thorough filling of the interstices between the surface fibres has been accomplished.

In order to produce a proper type of surface impregnum it has been found desirable, as indicated, to subject the coated paper surface to the action of hot calender rolls. This is particularly efficient when the composition contains resin and plasticizing agents in admixture with the cellulose ester. The hot calender treatment induces a superimpregnation of the fibres and tends to close up pores developed during the evaporation of solvents from the coating composition, thus increasing the resistance to seepage by grease.

Papers treated with a surface impregnum of the compositions disclosed herein may be readily fabricated to form paper cups, boxes, cartons, and other containers for food products. It is often advantageous to impregnate only one side of a paper, this being then cut and folded to form containers in which the impregnated grease resistance surface forms the interior of the container fabricated therefrom. Such a container has been found to be suitable for the packing and transportation of greasy food products such as bacon, butter, lard and other greasy articles.

The invention therefore involves a medium suitable for grease-proofing paper comprising substantially a grease-insoluble coating material and a composite solvent vehicle therefor. The invention further involves a composite solvent vehicle comprising solvents which are ordinarily very volatile but containing a modicum of wax which greatly reduces the evaporation of the solvent at room temperature, while permitting free evaporation thereof at slightly elevated temperatures. As heretofore stated the grease resistant material employed must comprise a grease-insoluble material as the basic ingredient and may contain plasticizers and various extending agents. The invention is concerned with

the process of hot calendering a paper carrying a cellulose ester surface impregnum resistant to penetration by oils and greases whereby increased resistance to said penetration is obtained. The invention comprises not only paper carrying a surface impregnum of said grease-resistant materials, but also paper containers (cartons and the like) made therefrom.

#### Example 3

|                                     | Parts by weight | 75 |
|-------------------------------------|-----------------|----|
| Nitrocellulose                      | 30              |    |
| Cottonseed phthalic glyceride resin | 160             |    |
| Acetone                             | 250             | 80 |
| Mineral wax                         | 2               |    |

#### Example 4

|                                     | Parts by weight | 85 |
|-------------------------------------|-----------------|----|
| Nitrocellulose (low viscosity)      | 40              |    |
| Cottonseed phthalic glyceride resin | 400             |    |
| Ethyl acetate                       | 200             |    |
| Acetone                             | 200             |    |
| Benzol                              | 300             | 90 |
| Wax                                 | 15              |    |

Owing to the high proportion of resin in Examples 3 and 4, it may be necessary to pass the coated paper over a hot plate immediately before folding into cartons, since the heated paper may be bent to better advantage than when cold. Preheating before folding allows of the use of a relatively high proportion of resin.

If the resin were not grease-proof so high a proportion would be unsafe, but is feasible with a grease-resistant resin of the type specified in Examples 2, 3 and 4.

In a similar manner peanut oil phthalic glyceride may be employed in Examples 2, 3 and 4 in complete replacement or partial substitution of the cottonseed product.

The glycols, such as ethylene or propylene glycols may be used to form synthetic balms which are appropriate for use with nitrocellulose especially in conjunction with resins of the type particularly noted above. Thus I may employ for coating the carton board the following:

#### Example 5

|                                            | Parts by weight | 110 |
|--------------------------------------------|-----------------|-----|
| Nitrocellulose (4 second viscosity)        | 20              |     |
| Soya bean oil benzoic glycol balm          | 35              |     |
| Solvent mixture (ethyl acetate and benzol) | 200             | 120 |
| Paraffin wax                               | 2               |     |
| Ceresin wax                                | 2               |     |

#### Example 6

To the composition of Example 5 add 50 parts cottonseed phthalic glyceride and sufficient solvent to render of proper coating consistency.

*Example 7*

|                                           | Parts by weight |
|-------------------------------------------|-----------------|
| Nitrocellulose (2 second viscosity) ----- | 30              |
| Oleic phthalic glycol-ether balsam -----  | 50              |
| Oxy rosin ester -----                     | 10              |
| Acetone -----                             | 10              |
| Denatured alcohol -----                   | 400             |
| Benzol -----                              | 5               |
| 10 Wax -----                              | 5               |

Example 7 contains a balsam of a different type, being made from a glycol-ether.

*Example 8*

|                                      | Parts by weight |
|--------------------------------------|-----------------|
| 15 Cellulose acetate -----           | 10              |
| Compatible glycol-ether balsam ----- | 20              |
| Solvent as in Example 7 -----        | 200             |
| Paraffin wax -----                   | 4               |

20 This composition may be used when the inflammability of nitrocellulose is considered a hazard.

*Example 9*

|                                                 | Parts by weight |
|-------------------------------------------------|-----------------|
| 25 Nitrocellulose (high viscosity) -----        | 10              |
| Rosin cottonseed phthalic glyceride resin ----- | 50              |
| 30 Tricresyl phosphate -----                    | 10              |
| Precipitated magnesium hydrate -----            | 10              |
| Hydrated calcium sulphate -----                 | 15              |
| Solvent as in Example 7 -----                   | 200             |
| Paraffin wax -----                              | 4               |

35 A coating of greatly reduced inflammability is secured by high resin content, use of tricresyl phosphate as a plasticizer and employment of hydrated inorganic bodies. The magnesium and calcium compounds used 40 in the above example have very slight hiding power, hence being of low pigment value yield a coating that is practically transparent if so desired.

Resins and balsams made with a phthalic 45 component have been referred to frequently in the foregoing for the reason that phthalic acid or anhydride is readily obtainable cheaply in abundant quantities and lends itself to resinification readily, but such illustrative 50 use of a desirable commercially-feasible form of resin is not to be construed as limiting the invention in any way as numerous other acids and anhydrides such as diphenic, terephthalic, salicylic, benzoic, chlor benzoic, 55 nitro benzoic, malic, maleic, succinic, sebacic, and the like, may be employed in producing a grease-resisting resin for the purposes of the present invention.

The process of the invention is illustrated 60 as follows:

*Example 10*

Carton board is fed from a roll through a coating device containing a coating composition such as is set forth above. Only one side 65 of the board is coated. The excess composi-

tion is removed from the surface by means of a scraper or doctor and the web travels through a steam-heated chamber in which the temperature is maintained at 135-140° F. An exhaust pump or blower attached to the hot chamber withdraws the solvent vapors. The web then passes to a hot roll or calender where the final surface solidification or compacting occurs. In this step any traces of residual solvent depart after having assisted in slightly softening or fluxing the surface impregnum, to the extent necessary to consolidate and integrate such impregnum. By carrying out the calendering at a temperature above the melting point of the wax, the latter tends to fill any porosities of the surface and assists in waterproofing the paper. This is of especial importance in the case of foods such as butter, mayonnaise and various emulsion products, as grease-resistance and water-resistance are required. The wax also acts as a lubricant, permitting the hot-calendering to proceed smoothly.

By the use of wax, the fire hazard from the employment of volatile inflammable solvents is greatly reduced, but in some cases the solvent itself must be of a slightly inflammable or non-inflammable character. To meet this requirement paper may be coated as follows:

*Example 11*

|                                           | Parts by weight |
|-------------------------------------------|-----------------|
| Low viscosity nitrocellulose -----        | 40              |
| Cottonseed phthalic glyceride resin ----- | 40              |
| Tricresyl phosphate -----                 | 20              |
| Carbon tetrachloride -----                | 100             |
| Butyl acetate -----                       | 170             |
| Paraffin wax -----                        | 5               |

The preferred form of finished carton board carries a scarcely-visible, flexible, grease-resistant surface impregnum comprising a cellulose ester, a grease-resistant substance and a wax. Heavier surfacings may be employed, but usually are not necessary and are more costly.

What I claim is:—

1. Glassine paper carrying a coating of a composition containing a cellulose ester, a wax in an amount sufficient substantially to reduce volatility of solvents for the composition but insufficient to cause substantial blemishing of the coating, and polyhydric alcohol-polybasic acid resin, the ingredients being in amounts sufficient to give substantial grease repellent properties to the paper.

2. Glassine paper carrying a coating of a composition consisting primarily of nitrocellulose, wax in an amount sufficient materially to reduce volatility of solvents for the composition but insufficient to cause substantial blemishing of the composition, and polyhydric alcohol-polybasic acid resin, the in-

gredients being in amounts sufficient to give grease repellent properties to the paper.

3. Glassine paper as defined in claim 1 in which the coating has been subjected to hot 70  
5 calendering subsequent to its application.

4. Glassine paper carrying a coating as defined in claim 2 in which the coating has been hot calendered subsequent to its application.

5. Glassine paper carrying a coating of a 10 composition consisting primarily of nitrocellulose, wax and polyhydric alcohol-polybasic acid resin, the ingredients being in amounts sufficient to give substantial grease repellent properties to the paper.

15 6. Glassine wrapping paper for covering greasy articles, said paper carrying a coating of a composition containing cellulose ester, wax and a resin of polyhydric alcohol-polybasic acid, the ingredients being in 80  
20 amounts sufficient to give substantial grease repellent properties to the paper.

7. Glassine wrapping paper for covering greasy articles, said paper having a coating of a composition consisting primarily of nitrocellulose, paraffin wax and polyhydric alcohol-polybasic acid resin, the ingredients being in amounts sufficient to give substantial grease repellent properties to the paper. 90

8. A glassine wrapping paper for covering 30 greasy articles, said paper carrying a coating of a composition consisting primarily of nitrocellulose, paraffin wax in an amount sufficient materially to reduce volatility of solvents for the composition but insufficient to 35 cause substantial blemishing of the composition, and polyhydric alcohol-polybasic acid resin, the ingredients being in amounts sufficient to give substantial grease repellent properties to the paper, the coating having 40 been hot calendered subsequent to its application. 100  
105

9. Glassine paper for wrapping greasy articles, said paper carrying a coating of a composition containing cellulose ester, paraffin wax in an amount sufficient substantially to reduce volatility of coating composition solvents but insufficient to cause substantial blemishing of the coating, and polyhydric alcohol-polybasic acid resin, the ingredients 45  
50 being in amounts sufficient to give substantial grease repellent properties to the paper, the coating composition having been subjected to hot calendering subsequent to its application. 110  
115

10. A covering for a grease containing article 55 consisting of a paper which is coated with a material consisting primarily of nitrocellulose admixed with a polyhydric alcohol-polybasic acid resin and wax, the materials being present in an amount sufficient to 60  
65 impart substantial grease repellent properties to the paper. 120  
125

11. A covering for a grease containing article consisting of a paper which is coated with a material consisting primarily of nitrocellulose admixed with a polyhydric alcohol- 130

polybasic acid resin and mineral wax, the materials being present in an amount sufficient to impart substantial grease repellent properties to the paper, the wax being present in an amount sufficient to reduce volatility of solvents for the coating composition, but being in an amount insufficient to cause substantial blemishing of the coating. 70  
75

THEODORE F. BRADLEY.

80

85

90

95

100

105

110

115

120

125

130